

# United States Patent

[19]

Smith et al.

[11] 3,892,893

[45] July 1, 1975

[54] **FIBRE TREATMENT**

[76] Inventors: **Geoffrey Allan Smith**, Lynton Darnick, Melrose; **Richard Young**, 31 Craig Park Gardens, Galashiels, both of Scotland

[22] Filed: **Sept. 20, 1972**

[21] Appl. No.: **290,747**

[52] U.S. Cl. .... **427/352**; 8/115.6; 427/353

[51] Int. Cl. .... **B44d 1/44**

[58] Field of Search..... 117/65.2, 115.6, 139.5 A, 117/140

[56] **References Cited**

UNITED STATES PATENTS

|           |         |               |             |
|-----------|---------|---------------|-------------|
| 2,040,105 | 5/1936  | Ritzert ..... | 117/65.2    |
| 3,434,984 | 3/1969  | Hyland .....  | 117/139.5 A |
| 3,483,024 | 12/1969 | Roff .....    | 117/65.2    |

|           |        |                     |             |
|-----------|--------|---------------------|-------------|
| 3,510,452 | 5/1970 | Frotscher .....     | 117/139.5 A |
| 3,523,033 | 8/1970 | Verburg et al. .... | 117/65.2    |
| 3,561,998 | 2/1971 | Snyder .....        | 117/65.2    |
| 3,563,794 | 2/1971 | Moriga .....        | 117/139.5 A |
| 3,655,437 | 4/1972 | Becker .....        | 117/139.5 A |

Primary Examiner—William D. Martin

Assistant Examiner—Janyce A. Bell

Attorney, Agent, or Firm—Fidelman, Wolffe & Leitner

[57]

## ABSTRACT

Natural and artificial fibres are treated with a setting, shrink-resisting or embossing chemical, said chemical being in a liquid medium, by application of the liquid medium to the fibre in a ratio of between 0.5 to 1.0 and 3.0 to 1.0 liquid medium to fibre, weight for weight. The fibre, which is preferably in fabric form, is then pressed for not more than 30 minutes.

7 Claims, No Drawings

## FIBRE TREATMENT

This invention relates to the treatment of natural and artificial fibres, more particularly in garment form in setting, shrink-resisting and embossing processes.

Present known methods of treating both natural and artificial fibres with either immediate contact or padded medium techniques, comprise the application of chemical to fabric using a liquid to fibre ratio (wt. to wt.) of the order of 20 or 30 to 1.

The present invention involves treatment of such fibres using short liquid to fibre ratios, or liquor ratios, which are of the order of 0.5 or 3 to 1. When a chemical, dyestuff, finishing agent or indeed any substance is applied to fibre which is in any form, but in particular in fabric or garment form, the rate of action between chemical and fibre is increased if a short liquid to fibre ratio (liquor ratio) is used.

Thus, by application of short liquid to fibre ratios in the treatment of fibres, production time and subsequently costs are lowered.

According to the present invention there is provided a method of setting, shrink-resisting or embossing fibre comprising:

applying to the fibre a chemical which is in a liquid medium, the chemical being for setting, shrink-resisting or embossing, said liquid medium contained in a bath at a temperature between 25° and 45°C.

adjusting the quantity of liquid on the fibre until the ratio of liquid to fibre is between 0.5 to 1 and 3 to 1 weight for weight; and

pressing the fibre for not more than 30 minutes.

Preferably the fibre is pressed for not more than 30 minutes at a pressure of between 3 lbs. per square inch. and 100 lb. per square inch.

Said liquid to fibre ratios, known as short liquor ratios are used for the treatment of both natural and artificial fibres.

Short liquid ratios used with an immediate contact technique for fabric treatments such as, setting, embossing, or shrink-resisting on natural and artificial fibres requires that chemicals should be placed directly where required.

Furthermore short liquor ratios are also used with the so-called padded medium technique for the treatment of natural fibres. Padding out a fabric of natural fibres is performed through a media of viscous liquid which enables the fabric to contain twice or three times the fabric weight of solution without shedding surplus solution by normal solution flow.

Specific examples of fibre treatment using liquid to fibre ratios (wt. for wt.) between 0.5 to 1 and 3 to 1 will now be given, by way of example.

## EXAMPLE I

For embossing lambswool shrink-resisting fibre in fabric form with the padded medium technique:

A fabric is embossed using a liquid comprising sodium hydrogen sulphite, sodium tetraborate and a polymer such as that under the Trade Names "Hercosett 57" or "Synthappret L.K.F." which is retained on the fabric by a viscous liquid comprising a binder or additive. "Hercosett 57" is a cationic fiber reactive aqueous solution of a polyamide epichlorhydrin resin and "Synthappret L.K.F." is a prepolymer of an aliphatic polyurethane containing free isocyanate groups. The binder

or additive provides sufficient viscosity to retain the right amount of liquid for treatment.

Clean lambswool shrink-resisted fabric, that is fabric which is free from spinning oils, is wetted out in a bath containing liquid at a temperature of about 40°C. The liquid comprises:

|                                           |                  |
|-------------------------------------------|------------------|
| Sodium Hydrosulphite                      | 10 grammes/litre |
| Sodium Tetraborate                        | 5 grammes/litre  |
| 10 "Hercosett 57" including<br>10% solids | 20 c.c./litre    |

The quantity of liquid in the bath is such that the ratio of liquid to fabric is about 12 to 1. This is the so-called wetting out liquor ratio.

The fabric is immersed in the liquid in the bath for two minutes and then removed through squeeze rollers or hydro extractors which give an embossing liquid pick up of 100 percent on the weight of fabric. Thus, 20 the liquid to fabric ratio is 1 to 1.

An embossed design is then applied to the fabric which is pressed for approximately six minutes.

Excess chemicals are washed from the fabric using a detergent, soap/alkali mixture or solvent.

25

## EXAMPLE II

For embossing bleached Cashmere fabric (bleached for example using hydrogen peroxide) which is free from spinning oils: The fabric is wetted out in a bath 30 containing liquid at a temperature of about 35°C., the liquid comprising:

|                       |                 |
|-----------------------|-----------------|
| Sodium Metabisulphite | 1 grammme/litre |
| "Hercosett 57"        | 5 c.c./litre.   |

The fabric is immersed in the liquid for three minutes, the liquid to fabric ratio being 10 to 1 weight for weight, the wetted-out fabric is then removed and placed in a hydro extractor which gives an embossing liquid pick up of 80 percent by weight on the fabric. Thus, the liquid to fabric ratio is 0.8:1.

An embossed design is applied to the fabric which is pressed for three minutes.

Excess chemicals are removed from the fabric in similar manner to Example I.

## EXAMPLE III

For embossing lambswool shrink-resisted fabric which contains spinning oils and aids: The fabric is wetted out in a bath containing liquid at a temperature of about 30°C., the liquid comprising:

|                    |                 |
|--------------------|-----------------|
| Sodium Sulphite    | 5 grammes/litre |
| Sodium Tetraborate | 5 grammes/litre |
| 5 "Hercosett 57"   | 15 c.c./litre   |

The quantity of liquid in the bath is such that the ratio of liquid is about 15 to 1. After immersing in the liquid for two minutes, the fabric is placed in a hydro extractor until the embossing liquid pick up is 120 percent on the weight of the fabric. Thus the liquid to fabric ratio is 1.2 to 1.

The fabric is then treated in similar manner to Examples I and II, the fabric pressing time being ten minutes.

## EXAMPLE IV

For setting a fabric which is free from spinning oils:

The same liquid is used as in Example I, the liquid to fabric ratio in the immersion bath, being 10 to 1.

The fabric is immersed for three minutes and then placed in a hydro extractor to give a setting liquid pick up of 100 percent on the weight of the fabric, i.e. liquid to fabric ratio of 1 to 1 weight for weight. 5

The fabric is then placed on a smooth flat board and pressed for ten minutes.

Excess chemical is removed using detergent or a soap/alkali mixture or a solvent. 10

#### EXAMPLE V

For shrink-resisting fabric treatment by the immediate contact technique: Paper is coated with a liquid of a polyamide type resin (HERCOSETT 57), containing 15 Borax and Sodium Metabisulphite dispersed to give a homogeneous mixture.

This paper, when placed in contact with wet animal fibred fabrics to give a liquid to fabric ratio of between 0.5 to 1 and 3 to 1, will, under the influence of heat (steam) and pressure i.e. 3/100 lbs. per square inch for up to 15 minutes, allow the stabilization of the woven or knitted fabrics to be such that the claim "Machine Washable" can be made.

The fabric is then given normal wash off with water 25 or water containing detergency.

We claim:

1. A method of treating a wool textile material consisting of fibre or fabric which comprises:

immersing said material in a bath of a liquid medium 30 at a temperature of between 25° and 45°C., said liq-

uid medium comprising a treating agent consisting of member of the group consisting of a polyamide epichlorhydrin resin or a prepolymer of an aliphatic polyurethane containing free isocyanate groups;

adjusting the quantity of said liquid medium on said material until the ratio of liquid medium to textile material is between 0.5 to 1.0 and 3.0 to 1.0 weight for weight;

pressing the textile material for not more than thirty minutes at a pressure of between 3 pounds per square inch and 100 pounds per square inch;

washing off any excess medium from said textile material; and

recovering the treated textile material as the product of the process.

2. the method of claim 1 wherein the textile material is fabric.

3. The method of claim 1 wherein the textile material is fibre.

4. The method of claim 2 wherein the treating agent is polyamide epichlorhydrin resin.

5. The method of claim 2 wherein the treating agent is a prepolymer of an aliphatic polyurethane containing free isocyanate groups.

6. The method of claim 3 wherein the treating agent is polyamide epichlorhydrin resin.

7. The method of claim 3 wherein the treating agent is a prepolymer of an aliphatic polyurethane containing free isocyanate groups.

\* \* \* \* \*